

## UNITED STATES PATENT OFFICE

2,084,472

LUBRICATING AND INSULATING  
COMPOUND

Peter J. Wiezevich, Elizabeth, N. J., assignor to  
Standard Oil Development Company, a cor-  
poration of Delaware

No Drawing. Application July 14, 1934, Serial  
No. 735,204

12 Claims. (Cl. 87-9)

The present invention relates to improvements in lubricating and insulating compounds and more specifically to inorganic acid ester compounds. The present invention is a continuation in part of a prior application, Serial No. 690,770, filed September 23, 1933, and will be fully understood from the following description.

In the previous application referred to above certain inorganic acid esters, especially the aromatic phosphoric esters, were disclosed as safety lubricants, especially turbine oils, because in addition to the primary requisites such as viscosity, oiliness and the like, those materials are characterized by high flash and ignition temperatures. The same is also true of boric esters. Both of these classes of compounds are not only applicable as lubricants but also make excellent insulating oils for transformers, switches, substation type circuit breakers and the like.

The esters which are of the greatest value are the aryl, that is to say phenolic, esters of phosphoric and boric acids, particularly the alkylated aryl esters such as tri-ortho-cresyl phosphate, but the aliphatic esters are suitable as well.

One difficulty with these materials appears to be their tendency, at least in the technical or commercially available grades, to deteriorate at elevated temperatures, with formation of acidity, but it has now been found that this can be reduced to an unobjectionable degree by the addition of oxidation inhibitors.

Practically all types of inhibitors soluble in ester compounds are suitable for the present purpose and among those may be mentioned particularly the phenol types, especially the poly-hydroxy, monocyclic compounds, such as resorcinol, pyrogallol and the like, and the mono- or poly-hydroxy bicyclic aromatic materials such as the alpha or beta naphthols. Aromatic amino compounds are also satisfactory, such as the naphthyl amines. Aromatic sulphur compounds are also effective, such as thiophenols and naphthols, sulphides, disulphides and the various polysulphides. Ordinary ethers, but especially thioethers, containing at least one aromatic radical can be used and such radical may be either purely hydrocarbon or substituted, for example, containing a hydroxyl or amino group. The above will serve to illustrate the fact that all of the known types of inhibitors which are soluble in the ester compounds are suitable for the present purposes.

The amount of inhibitors will vary somewhat, depending on their inherent strength, but in all cases the amount is minute, for example as little

as 0.05% is often sufficient, but usually 0.1% will be used. In rare instances more than 0.5% may be employed but in practically all cases the amount used is less than 1%.

To illustrate the effect of the inhibitors on the oxidation of these esters the following tests may be considered:

Example 1

In this case the ester compound was tri-ortho-cresyl phosphate of a technical or commercial grade. Its specifications are as follows:

|                           |                   |
|---------------------------|-------------------|
| Viscosity @ 100° F.       | 132 sec. Saybolt  |
| Viscosity @ 210° F.       | 39.4 sec. Saybolt |
| Demulsibility             | 1620              |
| Pour point                | -20° F.           |
| Flash                     | 450° F.           |
| Auto ignition temperature | Above 1000° F.    |

The above product and the same to which had been added 0.1% of alpha thionaphthol were submitted to oxidation absorption tests. In these tests air is bubbled in a closed circuit through the oil (10 c. c. sample) while maintained at 200° C. at 15 minute intervals. The amount of oxygen absorbed is determined by the difference from the amount remaining.

| Sample                         | C. c. oxygen absorbed (10 c. c. sample) 15 minute intervals |     |                       |    |    |    |    |   |
|--------------------------------|-------------------------------------------------------------|-----|-----------------------|----|----|----|----|---|
|                                | 1                                                           | 2   | 3                     | 4  | 5  | 6  | 7  | 8 |
| Tri-ortho-cresyl phosphate     | 73                                                          | 272 | Too rapid to measure. |    |    |    |    |   |
| Same + .1% alpha thio naphthol | 11                                                          | 26  | 36                    | 17 | 16 | 14 | 12 | 9 |

Example 2

In another test the blank sample (300 c. c.) and the same containing .11% alpha naphthol were blown with air while at 300° F. at a rate of 10 cubic feet per hour. The acidity was measured at intervals and the data recorded in the table below:

| Sample                 | Acidity mg. KOH/gr. |        |         |         |
|------------------------|---------------------|--------|---------|---------|
|                        | 3 hrs.              | 6 hrs. | 24 hrs. | 75 hrs. |
| Blank                  | .26                 | .31    | 1.2     | 1.39    |
| Sample + .11% naphthol | .13                 | .13    | .27     | .54     |

These latter samples were also submitted to Sligh tests, the blank showing 6.5 mg. while the inhibitor reduced this to 1.6 mg. in the sample to which it was added.

To these inhibited esters may be added thickeners, soaps, sludge dispersers, bases, oiliness agents, extreme pressure lubricating agents and other known blending agents which may be desirable to adapt the material to some specific purpose.

The present invention is not to be limited by any theory of the mechanism of the inhibitor action or to any particular inhibitor or ester but only to the following claims in which it is desired to claim all novelty inherent in the invention.

I claim:

1. Composition of matter comprising an organic ester of an inorganic acid and not over 1% of an oxidation inhibitor selected from the class consisting of phenols, amino compounds, aromatic sulfur compounds, ethers and thio ethers containing at least one aromatic radical.

2. Composition according to claim 1 in which the ester contains aromatic nuclei comprising at least 50% of the weight of the ester.

3. Composition of matter comprising the organic ester of an acid selected from the group of phosphoric and boric and not over 1% of an oxidation inhibitor selected from the class consisting of phenols, amino compounds, aromatic sulfur compounds, ethers and thio ethers containing at least one aromatic radical.

4. Composition according to claim 3 in which the ester is a phenolic ester.

5. Composition according to claim 3 in which the ester is a phenolic ester of phosphoric acid.

6. Composition according to claim 3 in which the ester is tricresyl phosphate.

7. Composition of matter comprising tri-ortho cresyl phosphate and not over 1% of an oxidation inhibitor selected from the class consisting of phenols, amino compounds, aromatic sulfur compounds, ethers and thio ethers containing at least one aromatic radical.

8. Composition according to claim 7 in which the inhibitor is an aromatic compound containing a radical selected from the group of hydroxy and amino radicals.

9. Composition according to claim 7 in which the oxidation inhibitor is selected from the group of naphthols and naphthyl amines.

10. Composition according to claim 7 in which the inhibitor is an aromatic compound selected from the group of thiophenolic compounds, aromatic sulphides, disulphides and polysulphides.

11. Composition according to claim 7 in which the inhibitor is selected from the group of thiophenols and thionaphthols and sulphides, disulphides and polysulphides of aromatic hydrocarbons.

12. Composition according to claim 7 in which the inhibitor is thionaphthol.

PETER J. WIEZEVICH. 30